# EUROPEAN PATENT APPLICATION

(11) **EP 0 272 218 A2**
(43) Date of publication of application: **22.06.1988**
(21) Application number: 87810745.7
(22) Date of filing: 11.12.1987
(51) Int. Cl.: G03C 5/44, G03H 1/18

(54) **Method of preparing a hologram**

(30) Priority: 17.12.1986 GB 8630187
(71) Applicant: ILFORD Limited, Mobberley Knutsford Cheshire WA16 7HA (GB)
(72) Inventor: Groves, Trevor, Wincham Northwich (GB); Hopwood, Antony Ian, Withington Manchester M20 9DU (GB); Clark, John Andrew, Altrincham Cheshire WA15 9HY (GB); Briggs, Timothy Nigel, Sandbach Cheshire CW11 9BU (GB)

(57) **Abstract**

Method of preparing a hologram which is of the silver halide in gelatin binder type which method comprises holographically exposing, developing, and bleaching holographic materials by means of a rehalogenation bleach bath, which contains a water-soluble halide and a ferric salt of an acetic acid derivative. Holograms thus prepared exhibit less haze and stain.

## Description

This invention relates to a method of preparing a hologram.

To produce a phase hologram from holographic material which is of the silver halide in a gelatin type, the material is holographically exposed and is then developed in a silver halide development agent. The developed silver is then removed using either a solvent bleach bath or a rehalogenating bleach bath. When a solvent bleach bath is used the developed silver is converted to a soluble silver salt which is washed out of the material in a final washing. When a rehalogenating bleach bath is used the developed silver is converted to a silver halide. This silver halide is redistributed within the gelatin layer and it helps to reinforce the holographic image and to increase its diffraction efficiency.

The most commonly used silver bleaching agents to use in a rehalogenating bleach bath is a ferric complex of ethylene diaminetetraacetic acid (E.D.T.A) such as ferric ammonium E.D.T.A or ferric sodium E.D.T.A. However, the use of these complexes is not entirely satisfactory as the hologram produced tends to be hazy and to exhibit some stain.

We have found a method of preparing a hologram which provides less hazy holgrams than those obtained when ferric ammonium or ferric sodium E.D.T.A. is used to bleach the developed silver.

Therefore according to the present invention there is provided a method of preparing a hologram which is of the silver halide in gelatin binder type, which method comprises holographically exposing holographic material by use of a coherent light, developing the holographic image by use of a silver halide developing solution and then bleaching the developed silver by use of a rehalogenating bleach bath which comprises a water soluble halide and the ferric salt of diethylenetriamine pentaacetic acid, the ferric salt of nitrilotriacetic acid, the ferric salt of ethyleneglycol tetraacetic acid or the ferric salt of 1,3-propylene diamine tetraacetic acid or a mixture of said ferric salts.

The ferric salt of diethylenetriamine pentaacetic acid is hereinafter referred to as ferric DTPA.

The ferric salt of nitrilotriaacetic acid is hereinafter referred to as ferric NTA.

The ferric salt of ethyleneglycol tetraacetic acid is hereinafter referred to as ferric EGTA.

The ferric salt of 1,3-propylenediamine tetraacetic acid is hereinafter referred to as ferric PDTA.

These ferric salts can be used either individually or in a mixture of these salts.

Another object of the present invention is a rehalogenating bleach bath which comprises a water-soluble halide and said ferric salt or a mixture of said ferric salts.

The preferred water soluble halide to use in the bleach bath is a bromide such as potassium and sodium bromide, where potassium bromide is preferred. The preferred concentration of bromide is from 1.0 to 40.0 g/litre. Most preferably about 10 g/litre is used.

A useful concentration of the ferric compound to use in the bleach bath is from 10 g/litre to 90 g/litre. The preferred concentration is about 20 g/litre. The preferred pH range is from 1.0 to 4.0 and most preferably is about 2.0.

When the concentration of ferric compound is much below 10 g/litre the bleaching process takes longer. When more than 90 g/litre are used solubility problems arise if it is required to prepare concentrated solutions.

The following Examples will serve to illustrate the invention.

It is to be understood that a large number of other ferric salts of sequestering agents were also tried but apart from the above four listed salts the reduction in haze compared with ferric EDTA was not significant.

The following Examples will serve to illustrate the invention.

### Example I

Samples of holographic material were prepared by coating onto a transparent photographic film base a gelatino silver halide emulsion which was substantially pure silver bromide having a mean crystal size of 0.03 microns at a silver coating weight of 30 mg/dm². The emulsion was optically sensitised with a red sensitising dye so that it was optimally sensitive to 633 nm. to colour of a He:Ne laser.

The material was holographically exposed using a He:Ne laser by a Denisyuk exposure method using a brushed aluminium plate as an object to yield (after processing) a reflective hologram. The beam power of the laser was 400 µW/cm².

The material was developed for 2 minutes at 30°C in a solution of the following formulation:
Sodium Sulphite Anhydrous 30 g
Hydroquinone 10 g
Sodium Carbonate 60 g
Water to 1000 ml

The samples were then water washed for 30 seconds and then transferred to two rehalogenating bleach baths of the following formulae:

(Bath 1 is the comparative bleach bath, whilst Bath 2 is a bleach bath of use in the present invention).

The samples of holographic material were soaked in the bleach baths which were held at 30°C until all the silver had been bleached out. The samples were then washed in running water for 5 minutes and then air dried.

The following series of tests were made. The sets of holographic material were subjected to exposure times of 1/15 second, 1/8 second, 1/2 second and 1 second. Brightness measurement of the processed samples showed that the maximum diffraction efficiency was obtained when the length of exposure was 1/2 second. The percentage haze was then measured for the two sets of samples one which had been processed using bleach Bath 2. The percentage haze was measured for both sets of samples at 450 nm and at the peak absorption of the hologram which was 580 nm. The results are shown in Figure 1 which accompanies this application.

Figure 1 shows that the percentage haze present in the samples processed in Bath 2 is significantly less than those processed in Bath 1.

The silver bleaching time for the two sets of samples in both Bath 1 and Bath 2 were also measured. The results are shown in Figure 2 which accompanies this application.

From Figure 2 it can be seen that the bleaching time when using Bath 2 was significantly less than when using Bath 1.

Also it was noticed, but this is difficult to quantify, that at the higher exposure times, that is to say the 1/2 second and 1 second exposures, significantly more stain was observable in the holograms which were processed in Bath 1. Lack of stain is particularly important when the holograms are to be used as holographic optical elements (HOE's).

### Example II

Further samples of holographic material were prepared as in Example I. The samples were holographically exposed as in Example I except that the beam power of the laser used was 200 µW/cm².

The samples were then developed for 2 minutes at 30°C in a solution of the following formulation:
Sodium ascorbate 35 g
potassium carbonate 30 g
acetic acid 1.4 ml
water to 1 litre

The samples were then water washed for 30 seconds and then transferred to one of the following rehalogenating bleach baths.

### Baths 2-7:

All these baths contained 0.1 M ferric nitrate (9 H₂O)
0.1 M sequestering agent
10 g/litre potassium bromide
water 1 litre

The sequestering agent and the pH of the baths were as follows:

The samples of holographic material were soaked in the bleach baths which were held at 30°C until all the silver halide been bleached out. The samples were then washed in running water for 5 minutes and then air dried.

Haze measurements were made as in Example I on each sample. Thus the exposure was 1/2 second. The percentage haze was measured at 580 nm the peak absorption of the hologram.

Thus the rehalogenating bleach baths of the present invention when used to process holographic material yield considerably less haze in the processed hologram.

## Claims

1. A method of preparing a hologram which is of the silver halide in gelatin binder type, which method comprises holographically exposing holographic material by use of a coherent light, developing the holographic image by use of a silver halide developing solution and then bleaching the developed silver by use of a rehalogenating bleach bath which comprises a water soluble halide and the ferric salt of diethylenetriamine pentaacetic acid, the ferric salt of nitrilotriaacetic acid, the ferric salt of ethyleneglycol tetraacetic acid or the ferric salt of 1,3-propylene diamine tetraacetic acid or a mixture of said ferric salts.

2. A method according to claim 1 wherein the concentration of ferric compound present in the rehalogenating bleach bath is from 10 to 90 g/litre.

3. A method according to claim 1 wherein the concentration of ferric DTPA present in the rehalogenating bleach bath is about 20 g/litre.

4. A method according to claim 3 wherein the pH of the rehalogenating bleach bath is from 1.0 to 4.0.

5. A method according to claim 4 wherein the pH is about 2.0.

6. A method according to claim 1 wherein the water soluble halide present in the rehalogenating bleach bath is a bromide.

7. A method according to claim 6 wherein the bromide is potassium bromide.

8. A method according to claim 6 wherein the amount of bromide present is from 1 to 40 g/litre.

9. A method according to claim 8 wherein the amount of bromide present is about 10 g/litre.

10. A rehalogenating bleach bath which comprises a water soluble halide and the ferric salt of diethylenetriamine pentaacetic acid, the ferric salt of nitrilotriaacetic acid, the ferric salt of ethyleneglycol tetraacetic acid, or the ferric salt of 1,3-propylene diamine tetraacetic acid or a mixture of said ferric salts and which has a pH within the range 1 to 4.

11. A rehalogenating bleach bath according to claim 10 wherein the soluble halide is potassium halide.

12. A rehalogenating bleach bath according to claim 10 wherein the concentration of ferric salt is from 10 to 90 g/litre.
